

Oct. 26, 1954

F. L. BOSQUI ET AL

2,692,677

# PROCESS FOR CLASSIFYING MAGNETIZED OR MAGNETIZABLE SOLIDS

Filed Feb. 9, 1951

2 Sheets-Sheet 1



Oct. 26, 1954

F. L. BOSQUI ET AL

2,692,677

PROCESS FOR CLASSIFYING MAGNETIZED OR MAGNETIZABLE SOLIDS

Filed Feb. 9, 1951

2 Sheets-Sheet 2



FIG. 2.

INVENTORS:  
Francis L. Bosqui &  
Thomas D. Heath,  
By Arthur M. Madole  
ATTORNEY

## UNITED STATES PATENT OFFICE

2,692,677

PROCESS FOR CLASSIFYING MAGNETIZED  
OR MAGNETIZABLE SOLIDS

Francis L. Bosqui and Thomas D. Heath, Westport, Conn., assignors to The Dorr Company, Stamford, Conn., a corporation of Delaware

Application February 9, 1951, Serial No. 210,252

4 Claims. (Cl. 209—39)

1

This invention relates to closed-circuit grinding of ores and other solids. In this type of grinding, the ore, usually found in the form of a solid mass of a mixture of locked particles is supplied to a ball or other grinding mill the discharge of which is usually delivered to a classifier where the finely divided solids are segregated into fractions of which fines go into one fraction while coarse particles go into another fraction. The coarse particles so fractionated are returned to the mill for regrinding whereas the fines, being small enough, go to further treatment. This closed-circuit classification is quite satisfactory when the solids treated are not or do not become magnetically polarized, or, i. e. magnetized. But to date, it has been impossible commercially without demagnetization to classify in closed-circuit grinding systems solids, of which magnetite ores are examples, that are magnetically susceptible, after said solids have become magnetically polarized. In recent years, research has been carried on in an attempt to develop equipment for successfully carrying out the demagnetization step. Such modern equipment now in use includes complicated high frequency tunable generators connected to elaborate oscillatory coils which require a cooling medium of some kind. So it is an object of this invention to devise ways and means for grinding in closed circuit, such magnetically polarized solids, and especially magnetite or similar ores without demagnetizing the material. It is a further object to classify coherent magnetized ores into a coarse fraction and a fine fraction without first demagnetizing them.

The desired function of the classifier in a closed-circuit grinding system, is to separate the suspended solids in the mill discharge so that the larger or coarser solid particles are passed from the classifier as one fraction returning to the mill, while the finer solid particles, that are already ground fine enough, are passed from the classifier as another fraction that goes to further treatment. When the solids so treated have no constituent that is or can become magnetized the classification is satisfactory. But where the solids have some constituent which is or becomes magnetized, such as certain iron fractions, it becomes highly unsatisfactory. The reason is that there is enough magnetic effect between

5 coarse and fine particles so that their mutual magnetic attraction to each other is greater than the classifying effect of the classifier, with the result that the fines cannot be parted from the coarse in the classifier. This happens irrespective of the means by which the solids have become magnetized. In any case, the suspended solids going to the classifier are said to be coherent, namely, particles thereof are coherent to each other with a magnetic force greater than the force available in the conventional gravity type classifiers. So another object of this case is to devise ways and means for effectively and satisfactorily classifying or fractioning such solids into a coarse fraction and a fines fraction in spite of such magnetic mutual coherence.

10 Some solids, either natural or artificial, that have some magnetically susceptible constituent, are first given a rough concentrating step such as being passed through a magnetic separator or 15 cobber, prior to going to the classifier in the closed-circuit grinding system. Such a separator acts to magnetize any solids present which are capable of being magnetized even though they had not been previously magnetized, whereby the 20 solids magnetically cohere to one another. So it is another object of this invention to classify satisfactorily such cohering solids irrespective of whether they were naturally magnetized or became magnetized either in a magnetic separator or in any other way.

25 In summary, the above, and possibly other objects, are attained by passing the solids discharging from the grinding mill, such as a ball or tube mill, to a liquid cyclone at such feed pressure that sufficient shearing forces are set up within the hydrocyclone so that the clusters or aggregates of magnetically cohered particles are broken up and simultaneously the coarse particles are hydraulically separated from the fine particles. The 30 feed pressure must not be so great, however, that the shearing forces cause a substantial portion of the individual particles to be comminuted. The coarse particles leave the hydrocyclone through its apex discharge, while fines leave it from its base discharge. Any mutual coherent forces between particles are overcome and contact between the particles is broken by the hydraulic shearing effects set up in such a hydrocyclone, with the result that the desired fractionation 35 takes place.

A typical hydrocyclone so used comprises a conical section merging into a cylindrical section. The conical section has an outlet or discharge for coarse particles at its apex, while the cylindrical section has its top at what would be generally the base of the cone and in this base there is an outlet or discharge for fines. Suspension to be treated is fed to the hydrocyclone tangentially in the cylindrical section which normally has what is called a hollow vortex finder extending from the base that comprises the fines base discharge. The opening in the apex and in the base are co-axial through both of which extend an air-core around which fractionated fines flow axially of the hydrocyclone to discharge through the vortex finder while the coarse solids are forced by centrifugal force toward the periphery of the conical section from whence the fraction of them discharges from the apex of the cone more or less annularly around the air-core. The hydrocyclone comprises a swirling chamber, in which there is set up a differential velocity gradient of such magnitude that any given cluster of material will be subject to shearing forces which will tend to disintegrate the cluster into its component particles. This differential velocity gradient is such that the liquid nearest the outer wall of the container is moving at the slowest velocity, whereas the material somewhere near to the center of the container is moving at the greatest velocity. When the differential velocity gradient overcomes the magnetic coherence of the cluster, the particles therein act individually and then acting individually they are subjected to differential settling rates because of the tangential velocity. This tangential velocity results in a centrifugal force which accomplishes the classification. It might be said that this invention first gives the particles a capacity for independent movement and then classifies them into a coarse fraction and a fine fraction while in this state of independent movement. The rate of classification will increase as the centrifugal force to which the particles are subjected increases.

Reference is now made to the drawings for a specific embodiment of this invention; however, it is to be realized that the invention may be embodied in other specific forms without departing from the spirit or essential characteristics thereof. The present embodiment is therefore to be considered in all respects as illustrative and not restrictive as the scope of the invention is defined by the appended claims and all changes that fall within the meaning and range of equivalents of the claims are therefore intended to be embraced thereby.

In the drawings, Fig. 1 represents a flowsheet showing the method of treating magnetized or magnetizable particles, so that they can be classified without demagnetization.

Fig. 2 is an idealistic drawing of the hydrocyclone showing the course taken by the particles in the apparatus.

More specifically, in the drawings magnetized or magnetizable natural or artificial solids are supplied to a ball mill 11, in which they are ground to particles at least some of which are fine enough whereby magnetically susceptible solids are liberated. By way of example, a screen analysis of a typical embodiment of the material is presented later. From the ball mill the ground material is passed through line 12 to a magnetic separator 13, in which a primary separation is made to remove some of the nonmag-

netic materials from the ore. The primary magnetic concentrate coming from the magnetic separator 13 contains both coarse and fine magnetized particles, and also contains a considerable amount of gangue material which is intimately associated with the particles, usually the larger particles. In this condition it is normally impossible commercially to classify the materials into a fine fraction and a coarse fraction, because the magnetic characteristics cause the particles to strongly cohere to one another. In general, at this point the fines comprise free gangue and liberated, relatively pure iron ore, whereas the coarse particles are solids with relatively pure iron ore particles still locked together with the gangue; therefore, it is desirable to separate the fines from the coarse so that the coarse may be recycled in closed-circuit to the ball mill 11 for further grinding.

The primary magnetics concentrate from the magnetic separator 13 is passed through pipe 14 to pump 15, from which it is supplied under considerable pressure through pipe 16 to the hydrocyclone feed 17. This imparting of high pressure is essential for the next step which occurs. Suitable pressures are specifically disclosed later. The material enters the hydrocyclone 18 and is subjected to shearing forces which are so enormous that they cause the clusters of magnetically cohered particles to be broken up. This hydraulic disassociation is a temporary condition. While in this temporary condition of disassociation the hydrocyclone 18 causes the temporarily disassociated material to be hydraulically classified into a coarse fraction and a fine fraction. The fine fraction passes upwardly and out of the hydrocyclone through base discharge conduit 19. The coarse fraction passes downwardly and out of the hydrocyclone through apex outlet 20. After discharge from the hydrocyclone, the particles in each fraction will again cohere, but now they have been classified. It might be said that this step causes temporary disassociation simultaneously accompanied by permanent classification.

The fines passing upwardly out of the base discharge conduit 19 of the hydrocyclone 18 are carried through line 21 into magnetic separator 22 from whence they are subjected to the final finishing step and yield the finished magnetic concentrate through line 23. Any nonmagnetics which accompany the fines will be rejected through line 24.

The coarse material which is discharged through apex outlet 20 is passed through line 25, through which it is recycled to ball mill 11; here it is reground and passed through the same steps as previously outlined. The result of this operation is a magnetic concentrate being produced through line 23, which magnetic concentrate is of extremely high purity. The data are presented later in table form showing the results of several runs.

Fig. 2 shows an idealistic view of the paths taken by the particles once they enter hydrocyclone 18. The materials enter the hydrocyclone feed 17, which must be a tangential feed so as to create a swirling motion in cylindrical section 32. To assist this swirling motion and to prevent short-circuiting of the material upwardly through the upper end 34 of the cyclone, there is inserted a hollow vortex finder 35 which projects downwardly into the cyclone to such that its lower end 37 is at a point lower than that of the feed 17. After the material is swirling at great speed in cylindrical section 32, it then

passes downwardly through conical section 33 and in so descending it swirls in ever decreasing circular paths. In these paths the shearing forces which are created temporarily overcome the magnetic coherence of the particles, thus causing disassociation without demagnetization. In this disassociated condition the centrifugal force then further causes an internal classification within the cyclone such that the heavier and larger particles are thrown into a zone which will be located nearest the outermost shield of the hydrocyclone. The finer particles will be located in a zone which is concentric with that of the coarse particles but which is located nearer to the center of the hydrocyclone. As these materials reach the apex outlet 20 the finer materials in the center of the hydrocyclone then turn upwardly and still in the directional swirling motion pass upwardly and out of the hydrocyclone through vortex finder 35. In the center of this ascending column of fines there will be located an air-core 38. The fines pass upwardly into hood 39, from whence they are discharged through pipe 21 to magnetic separator 22, as is shown in Fig. 1.

The coarse material is discharged through apex outlet 20 and passes from the apex outlet as an annular spray. This material is recirculated through pipe 25 back to the mill as shown in Fig. 1.

#### EXAMPLE 1

An iron ore, roasted to the magnetite state and magnetized by primary concentration in a magnetic separator, was passed through a hydrocyclone having a 3" cylindrical diameter and having a 120° cone attached thereto. A 1/2" vortex finder was inserted through the uppermost portion of the cyclone. The cyclone apex measured 3 1/2". A feed rate of solids of 3630 pounds per hour at an entrance pressure of 23 pounds per square inch was used. The solids in the feed pulp analyzed 39.8% by weight. After treatment in the hydrocyclone, the solids in the liquid coming from the vortex finder analyzed 15.2% by weight, whereas the solids coming from the apex analyzed 63.0% by weight. Not only was a disassociated classification effected, but these data show that the material was also thickened. The screen analysis of the iron ore used for this run was as shown in Table I:

Table I

| Run | Mesh | Percent + Cumulative |              |                |
|-----|------|----------------------|--------------|----------------|
|     |      | Cyclone Feed         | Cyclone Apex | Cyclone Vortex |
| 1   | 48   | 1.17                 | 1.43         | -----          |
|     | 65   | 9.46                 | 11.47        | 0.60           |
|     | 100  | 23.5                 | 28.2         | 2.68           |
|     | 150  | 39.4                 | 46.5         | 7.95           |
|     | 200  | 50.1                 | 58.1         | 14.1           |

Circulating load=4.4-1.

From an analysis of the information shown in Table I, it can be seen that although a feed was used containing 50% of the material of a size larger than 200 mesh (Tyler), nevertheless the cyclone was able to produce a vortex discharged material containing only 14% of a size larger than 200 mesh.

Four other runs using a cyclone whose charac-

teristics were the same as previously described resulted in the information shown in Table II:

Table II

|    | Cyclone Run                        | 2     | 3     | 4     | 5     |
|----|------------------------------------|-------|-------|-------|-------|
| 10 | Cyclone Apex, inches               | 1 1/2 | 1/2   | 1/2   | 7/16  |
|    | Entrance Pressure, p. s. i. g.     | 23    | 20-21 | 20-21 | 20-21 |
|    | Feed Rate, lbs./hr. solids         | 3,260 | 3,160 | 3,240 | 3,180 |
|    | Percent Solids in Feed             | 40.5  | 42.3  | 42.5  | 43.5  |
|    | Percent Solids in Vortex Discharge | 16.7  | 23.7  | 24.5  | 27.6  |
| 15 | Percent Solids in Apex Discharge   | 62.0  | 64.4  | 65.8  | 67.6  |
|    | Apex Solids/Vortex Solids          | 4.1/1 | 2.3/1 | 2.1/1 | 1.1/6 |

The screen analysis of the material produced from the runs shown in Table II is shown in Table III:

Table III

| Run | Mesh | Percent + Cumulative |              |                |
|-----|------|----------------------|--------------|----------------|
|     |      | Cyclone Feed         | Cyclone Apex | Cyclone Vortex |
| 30  | 48   | 1.58                 | 1.96         | -----          |
|     | 65   | 6.47                 | 7.95         | 0.36           |
|     | 100  | 17.6                 | 21.5         | 1.74           |
|     | 150  | 32.1                 | 38.3         | 6.80           |
|     | 200  | 45.1                 | 52.7         | 13.6           |
| 35  | 48   | 1.51                 | 1.50         | -----          |
|     | 65   | 5.65                 | 10.6         | 0.46           |
|     | 100  | 15.6                 | 25.8         | 2.77           |
|     | 150  | 31.8                 | 40.0         | 11.0           |
| 40  | 200  | 45.1                 | 55.0         | 22.1           |
|     | 48   | 1.4                  | 1.49         | -----          |
|     | 65   | 4.5                  | 6.25         | 0.50           |
|     | 100  | 11.6                 | 16.0         | 2.98           |
| 45  | 150  | 24.2                 | 29.8         | 9.62           |
|     | 200  | 35.0                 | 43.3         | 19.3           |
|     | 48   | 1.46                 | 1.94         | -----          |
|     | 65   | 4.09                 | 6.2          | 0.56           |
| 50  | 100  | 9.80                 | 15.4         | 3.3            |
|     | 150  | 21.6                 | 29.3         | 10.4           |
|     | 200  | 32.6                 | 43.0         | 22.2           |

#### EXAMPLE 2

Another series of runs was made using a cyclone as shown in the drawings, that is, one containing a cone with a 20° angle. Magnetized iron ore (magnetite) concentrate was used. A feed pressure of 25 pounds per square inch and a solids concentration of 35% was used for the feed. The vortex finder was 1.38" and the apex valve 1 1/8". The results of two runs made through a cyclone of these characteristics is shown below respectively in Tables IV and V:

Table IV

#### RUN #6

| Mesh   | Feed Percent C+ | Apex Percent C+ | Vortex Percent C+ |
|--------|-----------------|-----------------|-------------------|
| 20     | 0.08            | 0.10            | -----             |
| 28     | 0.15            | 0.20            | -----             |
| 35     | 0.31            | 0.43            | -----             |
| 48     | 0.39            | 0.50            | -----             |
| 65     | 1.49            | 1.93            | -----             |
| 100    | 6.87            | 8.80            | 0.33              |
| 150    | 20.33           | 26.00           | 1.22              |
| 200    | 36.55           | 46.70           | 2.54              |
| (-200) | 63.42           | 53.30           | -----             |
| 325    |                 |                 | 8.78              |
| (-325) |                 |                 | 91.22             |
| Total  | 100.00          | 100.00          | 100.00            |

| Mesh   | Feed Per-cent C+ | Apex Per-cent C+ | Vortex Per-cent C+ |
|--------|------------------|------------------|--------------------|
| 20     | 0.08             | 0.16             | -                  |
| 28     | 0.16             | 0.31             | -                  |
| 35     | 0.25             | 0.46             | -                  |
| 48     | 0.41             | 0.77             | -                  |
| 65     | 1.48             | 2.74             | 0.04               |
| 100    | 6.57             | 11.68            | 0.70               |
| 150    | 18.30            | 30.60            | 4.08               |
| 200    | 31.05            | 49.00            | 10.43              |
| (-200) | 68.95            | 51.00            | -                  |
| 325    | -                | -                | 32.70              |
| (-325) | -                | -                | 67.30              |
| Total  | 100.00           | 100.00           | 100.00             |

From the data which is here presented it can be seen that there is disclosed a method for classifying magnetized iron ore which was normally unclassifiable. There is also disclosed a method of controlling the mesh of separation of the material. If a coarse separation is desired, then a cyclone must be used which has a relatively large angled or "flat" conical section. If a finer mesh of separation is desired, then a steeper cyclone, such as a 20° cone, may be used. A comparison of the data shown in Table I with that shown in Table IV reveals that the wide angled cyclone produced a vortex overflow containing particles 14% of which were larger than 200 mesh, whereas a small angled or steeper cyclone produced a vortex overflow containing only 2.54% particles with a size larger than 200 mesh. In general, in order to decrease the load on the closed-circuit grinding system the wider angled cyclones will be more desirable. Using the wide angled cyclone, resulting in the test data shown in Tables II and III, Cyclone Run 5, a magnetic concentrate was prepared which analyzed 51.7% Fe from a feed of crude ore which contained 36.8% Fe; the feed to the cyclone contained 43.5% Fe. However, if local conditions require a purer product of a finer particle size, this can be obtained from a cyclone with a steeper conical section than was used for the run resulting in Table I.

In this specification the separation has been indicated as occurring in an apparatus essentially containing a conical section. The desired result of this invention may also be attained according to the teachings herein by swirling the material in any sort of a space confined by a surface of revolution. It must be fed tangentially and the fines must discharge essentially axially at the feed end. The coarse material may discharge axially or peripherally at the opposite end of the enclosed space.

We claim:

1. The continuous process of hydraulically classifying magnetically cohered particles, which comprises the steps of temporarily hydraulically dissociating the particles; and, while they are temporarily so dissociated, by hydraulically segregating the particles into a fine particle fraction and a coarse particle fraction.

2. A continuous process of hydraulically classifying magnetically cohered particles, which comprises tangentially introducing a mixture of the particles and liquid into one end of a body of liquid enclosed in a space confined by a surface of revolution and having an axial outlet in the infeed end along with an outlet at the opposite end; temporarily hydraulically dissociating the magnetically cohered particles by swirling the liquid in the body at a pressure sufficient to

establish and maintain concentric swirls of liquid having different annular velocities whereby interfacial shearing forces are established and maintained of magnitude sufficient to overcome magnetic coherence between the particles but

5 insufficient to substantially comminute the particles; hydraulically segregating the particles while they are temporarily so dissociated into a fine particle fraction and a coarse particle fraction; withdrawing the fine particle fraction through the axial outlet at the infeed end of the body; and withdrawing the coarse particle fraction from the outlet at the opposite end of the body.

10 3. A continuous process of liberating and segregating magnetically susceptible solids from a solid mass of magnetically susceptible solids locked together with non-magnetically susceptible solids, which comprises the steps of grinding the mass into particles some of which are fine enough and others of which are not fine enough; temporarily hydraulically dissociating the magnetically cohered particles by establishing

15 and maintaining a body of liquid enclosed in a space confined by a surface of revolution, tangentially introducing a suspension of the liquid and the cohered particles into an end section of the body at a pressure sufficient to swirl the body of liquid in concentric swirls having different annular velocities, establishing thereby interfacial shearing forces of sufficient magnitude to overcome magnetic coherence between the particles but insufficient to substantially comminute the particles; hydraulically segregating

20 within the body the particles while they are temporarily so dissociated into a fine particle fraction and a coarse particle fraction; axially discharging the fine particle fraction from the infeed end of the body while discharging the coarse

25 particle fraction from the opposite end of the body; recycling a quantity of the discharged coarse particles to the grinding step until the particles are ground fine enough; and subjecting the discharged fine particle fraction to magnetic separation to remove magnetically susceptible solids from the non-magnetically susceptible

30 35 40 45

solids.

4. A continuous process of liberating and segregating magnetically susceptible solids from a solid mass of non-magnetically susceptible solids locked together with magnetically susceptible solids, which comprises the steps of grinding the mass into particles some of which are fine enough and others of which are not fine enough; magnetically removing magnetically susceptible particles from a substantial portion of the non-magnetically susceptible particles; temporarily hydraulically dissociating the magnetically cohered particles by establishing and maintaining a body of liquid enclosed in a space confined by a surface of revolution, tangentially introducing a suspension of the cohered particles into an end section of the body at a pressure sufficient to swirl the body of liquid in concentric swirls having different annular velocities, establishing thereby interfacial shearing forces of sufficient magnitude to overcome magnetic coherence between the particles but of insufficient magnitude to substantially comminute the particles; hydraulically segregating

50 55 60 65

within the body the particles while they are temporarily so dissociated into a fine particle fraction and a coarse particle fraction; axially discharging the fine particle fraction from the infeed end of the body while discharging the coarse particle fraction from the opposite

70 75

end of the body.

9

end of the body; recycling a quantity of the coarse particles to the grinding step until the particles are ground fine enough; and subjecting the discharged fine particle fraction to magnetic separation to remove magnetically susceptible solids from the non-magnetically susceptible solids.

References Cited in the file of this patent

UNITED STATES PATENTS

| Number    | Name     | Date          |
|-----------|----------|---------------|
| 2,377,524 | Samson   | June 5, 1945  |
| 2,388,471 | De Vaney | Nov. 6, 1945  |
| 2,468,586 | Braund   | Apr. 26, 1949 |
| 2,543,689 | Driessen | Feb. 27, 1951 |

10

| Number    | Name     | Date          |
|-----------|----------|---------------|
| 2,558,635 | Vedensky | June 26, 1951 |
| 2,573,192 | Fontein  | Oct. 30, 1951 |

OTHER REFERENCES

| Number  | Country       | Date         |
|---------|---------------|--------------|
| 627,423 | Great Britain | Aug. 9, 1949 |

FOREIGN PATENTS

|    |                                                                                                                                                                         |
|----|-------------------------------------------------------------------------------------------------------------------------------------------------------------------------|
| 10 | Canadian Mining Journal, vol. 71, No. 6, pages 68, 69, June 1950.                                                                                                       |
| 15 | Engineering and Mining Journal, June 1950, vol. 151, issue No. 6, pages 71, 72, 73 (Erickson & Heckenoff); ("Cyclone Separation May Be Solution for Fine Ore Problem"). |
| 15 | Journal of the South African Chemical Institute, June 1949, vol. II, No. 1, pages 29-58.                                                                                |